

W. L. COURSEN,  
MANUFACTURE OF ZINC OXID,  
APPLICATION FILED JUNE 28, 1920.

1,372,486.

Patented Mar. 22, 1921.



Fig. 5,



Fig. 6,



Walter Leslie Courses Inventor

By his Attorneys  
Pennell Davis Marvin & Edmonds

# UNITED STATES PATENT OFFICE.

WALTER LESLIE COURSEN, OF PALMERTON, PENNSYLVANIA, ASSIGNOR TO THE NEW JERSEY ZINC COMPANY, OF NEW YORK, N. Y., A CORPORATION OF NEW JERSEY.

## MANUFACTURE OF ZINC OXID.

1,372,486.

Specification of Letters Patent. Patented Mar. 22, 1921.

Application filed June 28, 1920. Serial No. 392,204.

*To all whom it may concern:*

Be it known that I, WALTER LESLIE COURSEN, a citizen of the United States, residing at Palmerton, in the county of Carbon, State of Pennsylvania, have invented certain new and useful Improvements in the Manufacture of Zinc Oxid; and I do hereby declare the following to be a full, clear, and exact description of the invention, such as will enable others skilled in the art to which it appertains to make and use the same.

This invention relates to the production of French oxid (*i. e.*, zinc oxid) by the retort volatilizing process.

In the production of French oxid by the retort volatilizing process, it is the common practice in the art to charge the retorts with broken up slabs of zinc which must be melted and brought to the volatilizing temperature before the oxid production can take place. The production of French oxid in this way is an intermittent operation, each charge being worked off before the next charge is introduced into the retort. As a result, the retorts can be operated at their maximum capacity during only a part of the time. This intermittent method of operation requires frequent cleaning of the retorts, while the retorts themselves not infrequently crack or fail and must be replaced, thus further decreasing the output of the furnace and increasing the labor and expense of operation. So also, such intermittent operation of the retorts is wasteful of fuel for the reason that the retorts must be heated during the time interval between the end of one operation and the beginning of the next, as well as during the preliminary period of melting the zinc and heating it to the required temperature, and also during the entire working-off operation, during the latter part of which the retort is operated at a greatly reduced capacity, owing to the progressively decreasing amount of molten zinc remaining therein.

The present invention relates to an improved method of producing French oxid according to which the operation is carried out in a substantially continuous manner and with greatly increased capacity of the retorts and production of oxid, as well as other advantages, which will more fully appear from the following description.

In the application of James A. Singmaster, Serial No. 370,082, filed March 31, 1920, there is described an improved method of producing French oxid by the retort volatilizing process according to which the operation is carried out in a substantially continuous manner. The process of the present invention involves a similar continuous operation, but involves an improvement upon or modification of the process of said prior application. According to the process described in said prior application, the volatilizing retort is charged with molten zinc, and further amounts of molten zinc are charged from time to time to make up for that which has been volatilized. According to the present invention the retort is charged with solid zinc, instead of with molten zinc, but the operation is carried out with the maintenance of a substantial body of molten zinc in the retort, to which the increments of solid zinc are added from time to time, so that a similar continuous operation is obtained to that which is obtained when the retort is kept supplied with further amounts of molten zinc.

In the practice of the present invention, a preliminary charge of zinc or spelter is charged into the retort and the retort is brought to the temperature required for the volatilizing operation. Thereafter, further amounts of solid zinc are added to the retort from time to time to make up for that which is volatilized, but such further additions of zinc are relatively small in amount and a substantial body of molten zinc is retained in the retort, so that the retort operation is continuous, and the oxid production is likewise of a substantially continuous character, except for the period of time required for melting the added zinc and again bringing the contents of the retort to the volatilizing temperature.

In the practice of the invention, it is advantageous to maintain a sufficient body of molten zinc in the retort so that the retort will operate at approximately its maximum working capacity and so that the additions of solid zinc from time to time will not result in undue cooling of the contents of the retort. With such a body of molten zinc in the retort, the zinc which is added will be rapidly melted and brought to the volatilizing tem-

perature, so that small increments of solid zinc can be added from time to time without seriously interfering with the continuity of the operation. The maintenance of a substantial body of molten zinc has the further advantage of equalizing any inequalities in the zinc which is added from time to time, thereby promoting the uniformity of the oxid produced. Thus, where lead is contained in the zinc charged, this lead can be held back in the retort and prevented from any objectionable amount of volatilization by maintaining a substantial body of zinc in the retort, whereas, if the charge were entirely worked off, as in common practice, volatilization of lead would take place. Accordingly, by maintaining a sufficient excess of zinc in the retort, inequalities in lead contained in the zinc charged will be neutralized and the lead can be made to accumulate in the retort. When the lead has thus accumulated to such an extent as to interfere with the desired uniformity and purity of the product, the lead-containing residue can then be withdrawn from the retort. Accordingly, by maintaining a sufficient excess of molten zinc in the retort, a product of high purity and great uniformity can be obtained even where the molten zinc charged contains varying amounts of lead.

In the preferred practice of the invention, the zinc is supplied in the form of sticks or bars of relatively small size, such that they can be readily charged into the retorts. These sticks or bars can be readily provided by casting molten zinc or spelter in specially designed molds, instead of casting in the form of slabs according to the present practice. By providing the zinc or spelter in the form of relatively small and uniform sticks, the operator is able to supply to the individual volatilizing retorts one or more sticks from time to time to make up for the zinc which has volatilized. These sticks, being of small size, are rapidly melted by the highly superheated body of molten zinc within the retorts.

The invention will be further illustrated by the following more detailed description of the preferred practice thereof, reference being had to the accompanying drawing which illustrates, in a somewhat conventional and diagrammatic manner, a furnace construction adapted for the practice of the invention.

In the accompanying drawing—

Figure 1 is a vertical longitudinal section of an oxid furnace;

Fig. 2 is a vertical transverse section of such furnace;

Fig. 3 is a vertical sectional view of one of the volatilizing retorts;

Fig. 4 is a transverse sectional view of one of the retorts showing the level of the charge therein;

Fig. 5 is a plan of a suitable form of mold; and

Fig. 6 is an enlarged cross-section of a suitable form of stick or bar of zinc or spelter.

Referring to the drawing, the furnace 1 may be of any suitable construction, for example, it may be a regenerative gas-fired furnace, and it has therein a series of volatilizing retorts 2, twenty in number in the furnace illustrated. In the operation of a regenerative gas-fired furnace, the supply of air and gas is reversed from time to time so that combustion takes place first from one end of the furnace and then from the other, the waste products of combustion serving to heat the regenerators alternately in the usual way.

The retorts 2 may be of any suitable construction. As illustrated in Figs. 2, 3 and 4, they have the usual dam 3 at one end and the usual opening 4 thereabove and are closed at the other end by a closure or luting 5 through which extends the pipe 6 for supplying the reducing gas. This pipe 6 has a door 7 through which the sticks of zinc can be introduced.

The sticks of zinc for charging the retorts can be made by casting molten zinc or spelter in special molds. One suitable form of mold is indicated in Fig. 5, this mold having a series of depressions 8 for casting a series of sticks or pigs. The molten zinc or spelter can be poured into the depression 9 and permitted to flow into the individual lateral depressions, in a manner similar to that used in casting pig iron. The individual sticks or pigs can then be broken off from the sow and used for charging the retorts. The sticks thus cast can vary somewhat in size and length. A suitable size is about 18 to 24 inches long and 1 to 2 inches in width and depth. Such a stick, of about 1½ inches in width and depth, is illustrated in cross-section in Fig. 6.

The zinc used in making the sticks may be spelter directly from the spelter furnaces or it may be molten zinc from some other source. The casting of the zinc, to form the sticks, by the use of a suitable finger mold of the character above described, will be readily understood without further description, being similar to the common methods of casting spelter in slabs except for the form of mold employed.

In the production of the French oxid, the retorts are externally heated to a temperature above the volatilization point of zinc but below the volatilization point of lead, iron, etc., and the retorts are kept filled with a reducing gas, such as clean producer gas introduced through the pipe 13. The introduction of this gas prevents premature oxidation of the zinc vapor and also assists in sweeping out the zinc vapor as fast as

it is formed, thereby promoting its formation. The zinc vapor and the producer gas combine with the oxygen of the air at the retort mouth, and the oxid thus produced 5 is collected in the usual way.

The individual retorts can be charged, at the outset, with a sufficient number of sticks of zinc to make up the required charge. These sticks will be first melted to form a 10 substantial body of molten zinc which will then be heated to the volatilizing temperature. Thereafter, from time to time, one or more sticks are added to each retort to make up for the zinc which has been volatilized. For best results, the level of the 15 molten zinc in the retort should not be permitted to fall too low, and further additions of zinc should be made from time to time to maintain the level at approximately the maximum working capacity of the retort. 20 Inasmuch as the molten zinc is at a temperature considerably above the melting point of the added zinc, this zinc will be rapidly melted and the charge will soon 25 again reach the necessary temperature for volatilization. For example, in the volatilizing retort which holds a charge of about 225 pounds of molten zinc, the individual sticks may have a weight of around 6 to 8 30 pounds, and it will be evident that such sticks will be soon melted after they are added to the molten zinc in the retort.

By maintaining a substantial body of molten zinc in the retort, there is a maximum 35 surface exposure for volatilization, and approximately the maximum contact surface between the molten zinc and the walls of the retort through which the heat is transferred. Effective heating of the molten zinc in the 40 retort and effective volatilization thereof are thus secured.

The retort is preferably filled to about the level indicated in Fig. 4, and further additions are made from time to time to prevent 45 the level from falling too low, so that the retort will be operated at approximately its maximum working capacity.

When it becomes necessary to clean a retort and remove the ashes or the residual 50 molten metal therefrom, the closure 5 can be broken away to permit this cleaning operation. The retort can then be again charged with sticks of zinc and the retort closed by luting with clay or other material 55 which will bake and form a solid closure by the time the solid zinc has melted.

By operating in the manner above described, it has been found that the producing 60 capacity of the retorts can be very greatly increased. It has thus been found that a regular furnace which will consume about 150 tons of metal per month, with the zinc charged cold into the retorts, and the retorts operated in an intermittent manner, 65 will consume as high as 210 tons or higher

per month, when the furnace is operated in a substantially continuous manner, according to the present invention, even though the zinc is charged cold into the retorts.

This greatly increased capacity and yield 70 is due, as I believe, to the approximately constant and maximum heat transfer through the retort walls, owing to the large contact area between the molten zinc and the heated walls of the retort, and to the 75 continuity of the operation with a substantial body of molten zinc in the retorts, to which the sticks of solid zinc are added, and by which they are rapidly melted. The 80 continuity of operation with a substantial body of zinc in the retorts, avoids the time lost in intermittent operations for completing the working off of the individual charges, cleaning the retorts, recharging the 85 retorts intermittently, and melting and bringing each successive charge to the volatilizing temperature.

The improved process of the present invention presents many of the same or similar advantages to those presented by the 90 process of said Singmaster application, Serial No. 370,082, to wit, the advantage of increased capacity and yield, together with high zinc recovery and low operating cost, prolongation of the life of the retorts with 95 resulting reduction in zinc losses, less frequent renewal of the retorts, increased economy and efficiency of fuel, reduction in the labor required in cleaning and replacing the retorts, less frequent cleaning of the retorts, 100 etc. The present invention presents the further advantage that the zinc charged into the furnace is in a form readily handled and readily regulated in amount. The operator can thus go from one retort to another, and charge one or more of the solid sticks of zinc into the retort. The present invention thus makes possible the charging 105 of solid zinc into the retorts in a simple and advantageous manner, while nevertheless 110 obtaining the advantages of continuity of operation, increased fuel economy, etc.

I claim:

1. In the production of French oxid by the retort volatilizing process, the improvement which comprises maintaining a substantial body of molten zinc in the retort and adding further amounts of solid zinc thereto from time to time to make up for that which has been volatilized. 115

2. In the production of French oxid by the retort volatilizing process, the improvement which comprises operating the retort in a substantially continuous manner and at approximately the maximum working 120 capacity of the retort by maintaining a substantial body of molten zinc in the retort and adding further amounts of solid zinc thereto from time to time to make up for that volatilized. 125

130

3. In the production of French oxid by the retort volatilizing process, the improvement which comprises maintaining a substantial body of molten zinc in the retorts and adding thereto from time to time further amounts of zinc in the form of relatively small sticks or bars which are readily melted by the molten zinc in the retorts.
4. In the production of French oxid by the retort volatilizing process, the improvement which comprises maintaining in the volatilizing retort a substantial body of molten zinc having a large contact surface with the walls of the retort, and supplying to the retort from time to time further amounts of zinc in the form of relatively long and small sticks or rods, whereby effective heat transfer takes place through the

walls of the retort to the molten zinc therein and the added zinc is rapidly melted 20 thereby.

5. In the production of French oxid by the retort volatilizing process, the improvement which comprises maintaining a substantial body of zinc in the volatilizing retorts, adding thereto from time to time further amounts of lead-containing zinc in solid form, maintaining a sufficient excess of zinc in the retorts to hold back lead from volatilizing and thereby permitting lead to 25 accumulate in the retort, and finally withdrawing the residue rich in lead from the retort.

In testimony whereof I affix my signature.

WALTER LESLIE COURSEN.